



## U.S. PATENT DOCUMENTS

|                 |         |                      |
|-----------------|---------|----------------------|
| 5,415,921 A     | 5/1995  | Grohman              |
| 5,482,667 A     | 1/1996  | Dunton et al.        |
| 5,571,581 A     | 11/1996 | Koizumi et al.       |
| 5,615,523 A     | 4/1997  | Wells et al.         |
| 5,630,305 A     | 5/1997  | Hlasnicky            |
| 6,112,492 A     | 9/2000  | Wells et al.         |
| 6,303,224 B1    | 10/2001 | Krahn et al.         |
| 6,349,961 B1    | 2/2002  | Colley et al.        |
| 6,368,093 B1    | 4/2002  | Vecchiarino et al.   |
| 6,440,524 B2    | 8/2002  | Valyi et al.         |
| 6,536,177 B1    | 3/2003  | Italiene et al.      |
| 6,808,785 B1 *  | 10/2004 | Friedman et al. .... |
| 7,351,462 B2 *  | 4/2008  | Friedman et al. .... |
| 2003/0054148 A1 | 3/2003  | Jolitz et al.        |
| 2004/0148874 A1 | 8/2004  | Jolitz et al.        |
| 2004/0148895 A1 | 8/2004  | Jolitz et al.        |
| 2004/0177596 A1 | 9/2004  | Jolitz et al.        |

|                 |         |                 |
|-----------------|---------|-----------------|
| 2004/0178532 A1 | 9/2004  | Jolitz et al.   |
| 2004/0241476 A1 | 12/2004 | Friedman et al. |
| 2005/0086907 A1 | 4/2005  | Jolitz          |

## OTHER PUBLICATIONS

Mira Vista Shake Shingles Date Apr. 27, 2007 Believed to be the subject of U.S. patents 5,615,523 and 6,112,432, which appear to not have a capstock layer.

ES Report ER-5209 (3 pgs) Reissued Apr. 1, 2002. Believed to be the subject of U.S. patents 5,615,523 and 6,112,432, which appear to not have a capstock layer.

Mira Vista Shake and Slate Application Instructions Publication No. 15-RR-44159 Believed to be the subject of U.S. patents 5,615,523 and 6,112,432, which appear to not have a capstock layer.

Mira Vista Statement With Analysis (9pgs).

\* cited by examiner



## 1

## SYNTHETIC ROOFING SHINGLE OR TILE

## CROSS-REFERENCE TO RELATED APPLICATIONS

This is a continuation-in-part of application Ser. No. 11/531,788 filed Sep. 14, 2006, now U.S. Pat. No. 7,351,462, which is, in turn, a continuation of application Ser. No. 10/452,059 filed Jun. 2, 2003 now abandoned.

## BACKGROUND OF THE INVENTION

In the art of making roofing shingles and tiles for exterior application in the building industry, such products are made by compression molding of multi-component formulations, which comprise blends of virgin and recycled polymers and various low cost fillers.

In order to achieve low production costs, it is commonplace for manufacturers to use inexpensive raw materials, such as recycled resin of low quality with a very large amount of inexpensive filler derived from various waste streams. Such filler can include carbon black, recycled rubber tire crumb, coal fines, pulp and paper waste, and other inexpensive materials.

The use of large quantities of such fillers reduces the mechanical properties of the ultimate product, however. Additionally, the use of such large quantities of fillers limits the color variations that are possible in the products and makes the processing of the formulations into shingles and other exterior application building products very difficult.

Typically, roofing shingles and tiles made of such material having waste for filler do not provide good weather resistance for the products. Additionally, the warranty periods that can reasonably be provided for such products tend to be short in duration.

Furthermore such building industry roofing products have relatively low impact strength, especially at low temperatures. Insofar as their available colors are concerned, such tend to be limited to the colors gray and black.

## SUMMARY OF THE INVENTION

The present invention is aimed at providing for synthetic fabrication of roofing shingles or tiles for exterior application which are free of the above-mentioned deficiencies of the prior art.

The present invention involves a roofing shingle or tile for exterior application in the building industry, of synthetic material, comprising a core of inexpensive material weather-exposed portions of which are encapsulated by a skin of a different material, preferably of a polymer having high weather resistance and the ability to be colored in various colors. The core material will generally be of greater thickness than that of the skin material.

The skin material is melted and molded in some manner, and cools and solidifies, and the less expensive but greater volume of molten core material is also molded, but is disposed inside the skin and both are allowed to cool and solidify, such that a core of less expensive material has weather-exposed portions or surfaces encapsulated by a skin of greater quality, having high weather resistance, color acceptance, and other beneficial features, such as good impact resistance, longer lifetime warranty capability and, optionally, various surface design configurations.

The skin and core materials can be co-injected into the same mold cavity. Alternatively, the skin material and core material can be co-extruded from melted ingredients con-

## 2

tained within different cavities of a mold, so that the skin material encapsulates surfaces of the core material such that the skin material and core material are laminated together. Also, alternatively, the core material and skin material can each be compression molded and laminated together. Other alternative processes include co-extrusion followed by stamping or embossing blow molding of the skin and core materials, or rotational or sequential molding.

Regardless of the method of making the composite skin-and-core roofing product, three dimensional relief can be built into the mold cavity configuration or applied in a post-molding stamping or embossing operation to be present in the skin, in order to simulate various natural materials such as wood shales, tile, slate, etc.

Accordingly, it is an object of this invention to provide a multi-layer molded synthetic roofing shingle or tile, wherein a high quality thermoplastic skin layer of material encapsulates a plurality of surfaces of a lesser quality thermoplastic core layer of material, wherein each layer includes filler material to reduce material cost.

It is a further object of this invention to accomplish the above object, wherein the core material for the product is essentially a waste or recycled material.

It is a further object of this invention to accomplish the above objects, wherein the core material comprises the greater amount of material used in making the roofing shingle or tile.

Other objects and advantages of the present invention will be apparent from a reading from the following brief descriptions of the drawing figures, the detailed descriptions of the preferred embodiments, and the appended claims.

## BRIEF DESCRIPTIONS OF THE DRAWING FIGURES

In the drawings:

FIG. 1 is a top perspective view of synthetic roofing shingle or tile in accordance with this invention.

FIG. 2 is a transverse sectional view taken through the illustration of FIG. 1 generally along line II-II of FIG. 1, wherein the skin material is shown encapsulating the top surface and side edge surface of the core of the article illustrated in FIG. 1.

FIG. 3 is a fragmentary longitudinal sectional view taken through the illustration of FIG. 1, generally along the line III-III of FIG. 1, wherein the skin material is shown encapsulating the top surface and lower edge surface of the core of the article illustrated in FIG. 1.

FIG. 4 is a perspective view of a roof, partially covered by a plurality of shingles made in accordance with the shingles of FIGS. 1-3.

## DETAILED DESCRIPTIONS OF THE PREFERRED EMBODIMENTS

Referring now to the drawings in detail, reference is first made to FIG. 1, wherein a roofing shingle or tile 10 is illustrated, in the form of a rigid synthetic roofing shingle or tile. Such article 10 is typically illustrated as having upper and lower surfaces 11 and 12, right and left edge surfaces 13 and 14, and top and bottom edge surfaces 15 and 16. The article 10 may take on various other configurations as may be desired, other than the flat configuration shown. Typically, if it is to be made in the form of a tile, it may be flat or it may have a rounded or arched configuration. One or more ends such as that 16 may be of various other configurations, such as segmented, scalloped or the like, all as may be desired. One or

more surfaces **11** may have lines, grooves or seemingly random relief areas **19**, all as may be desired, for example to give the appearance of natural material, such as a cedar shingle, tile, slate, etc.

In general, the configurations of the various surfaces of the roofing shingle or tile **10** are unlimited as are the sizes of the same, within conventional sizes of shingles or tiles, as are shown, for example in FIG. 4, that lend themselves to be laid up on a roof, in courses, with a plurality of shingles or tiles in each course.

With reference to FIG. 2, it will be seen that the article **10** is comprised of a skin **18** and a core **20**, with the skin **18** encapsulating the top surface **21** of the core and forming encapsulating surfaces **13**, **14** and **16** of the edges that would be weather-exposed.

In FIG. 4, a plurality of shingles or tiles **10** are shown applied as a roof covering **32** to a roof **30** of a structure **31** with lower surfaces **12** being disposed against the roof surface **30** and therefore being not weather-exposed and therefore not needing a protective skin material **18** encapsulating surfaces **12**. Top edges **15** are likewise not weather-exposed because of next-overlying shingles covering such edges **15**, so skin-encapsulation is not necessary. Right, left and especially bottom edge surfaces **13**, **14** and **16**, respectively, are weather-exposed and are therefore skin-encapsulated.

The roof covering **32** as shown in FIG. 4 is seen to comprise a plurality of roofing elements **10**, toward the bottom of the roof **30**, laid up side by side to form a lower course **33**, with the next-overlying course **34** of such elements partially covering the roofing elements in the underlying course **33**, with a next overlying course **35** of such elements likewise partially covering the roofing elements in the underlying course **34**, followed by a next-overlying course **36** partially covering roofing elements in the next-underlying course **35**, and with a next-overlying course **37** of elements partially covering the roofing elements in the next-underlying course **36** of elements. Each of the elements **10**, comprising shingles or tiles, in each course are shown to be laid-up side-by-side, in FIG. 4. It will thus be seen that the process by which the various courses are applied in FIG. 4, are such that a lower-most course is first applied, followed by the application of a next-overlying course, with succeeding courses being applied partially covering next-underlying courses, in manner shown in FIG. 4 as the various courses are applied to form a roof covering **32**.

The core material **20** will generally be of greater thickness "T1" than the skin material **18** and will preferably be comprised of a highly filled polymer. The skin material **18** will preferably be comprised of a polymer having high weather resistance and the ability to be colored in various colors as may be demanded by building designers.

By combining a skin material **18** with a core material **20**, such allows an economic advantage in that a greater amount of filler may be used to comprise the core **20**, which will be of less expense than the material that comprises the skin, without providing undesirable surface properties for the skin, and without limiting the aesthetics of the product, because the core **20** is encapsulated in an aesthetically pleasing and weatherable skin **18**. Additionally, the core **20** can be comprised of a foam material where reduced weight for the product is desired.

In some embodiments the shingle or tile is comprised of a core **20** that is made of a low molecular weight material such as polypropylene tilled with 40-80% by weight of recycled ash with suitable functional additives, encapsulated in a skin **18** comprised of a film.

Such fillers as core material can vary considerably and can be chosen from a group that includes treated and untreated ashes from incinerators of power stations, mineral fillers and their waste, pulp and paper waste materials, oil shale, reclaimed acrylic automotive paint and its waste and/or mixtures of any of these.

The skin can be chemically cross-linked to increase its mechanical properties and weather resistance and/or flame resistance and can contain functional additives such as pigments, UV light stabilizers and absorbers, sensibilizers (photo-initiators), etc. The cross linking may occur during or after processing of the material.

By way of example, the skin material **18** is selected from a group of thermoplastic materials comprising Polyolefins such as Polyethylene (PE), Polypropylene (PP), Polymethylpentene (PMP) and Polybutene (PB-1), their copolymers, blends, and filled formulations, other polymers having high weather resistance such as Polyacrylates and/or their copolymers blends and filled formulations. The skin material is preferably stabilized for UV-light and weathering resistance by using additives and additive packages known in the state-of-the-art to be efficient. In addition, the skin materials may also contain various additives such as thermal and UV-light stabilizers, pigments, compatibilizers, processing aids, flame retardant additives, and other functional chemicals capable of improving processing of the materials and performance of the product. Foaming agents such as azodicarbonamide may be used to reduce the density of the skin material. Such polymers, with one or more additives, are therefore polymeric materials.

By way of example, the core material **20** may be selected from the group comprising of virgin thermoplastic polymer materials and elastomers and rubber including but not limited to Polyvinylchloride (PVC), Polyethylene (PE), Polypropylene (PP) Polybutene (PB-1), Polymethylpentene (PMP), Polyacrylates (PAC), Polyethyleneterephthalate (PET), Polybutyleneterephthalate (PBT), Polyethylenenaphthalate (PEN), Ethylene-Propylene-Diene Monomer Copolymers (EPDM), their copolymers, binary and ternary blends of the above, and filled formulations based on the above and other thermoplastic materials and elastomers with mineral, organic fillers, nanofillers, reinforcing fillers and fibers as well as recycled materials of the above polymers. Such polymers, with one or more additives, are therefore polymeric materials.

From the costs point of view, recycled and highly filled thermoplastic materials and recycled rubber (for example from tires) are preferable. The content of mineral fillers can be in the weight range from 5% to 80%.

In addition, the core materials may also contain various additives such as thermal and ultraviolet (UV) light stabilizers, pigments, compatibilizers, processing aids, flame retardant additives, and other functional chemicals capable of improving processing of the materials and performance of the product. Foaming agents such as azodicarbonamide may be used to reduce the density of the core material.

As indicated above, the skin **18** may, if desired, be embossed or stamped after the material is processed and the item is shaped, or the same may be molded to have relief portions to simulate embossing or stamping, during the molding process.

In making the products of this invention, the combined upper and lower layers **11** and **12**, of the skin **18** may comprise from 1% to 40% of the total thickness of the product, with the core **20** inside the skin **18** being thicker between surfaces **11** and **12** and comprising the remaining percentage of the total thickness "T" of the product.

It will be apparent from the foregoing that various other modifications may be made in the details of making the roofing shingle or tile of this invention, all within the spirit and scope of the invention as defined in the appended claims.

What is claimed is:

1. A rigid synthetic roofing element of a shingle or tile type, for exterior application, comprising a multi-layer structure having:

- (a) a skin including a first thermoplastic material;
- (b) a core including a second thermoplastic material;
- (c) wherein the first material is a highly weather resistant polymeric material relative to the second material;
- (d) wherein the second material is a polymeric material having filler therein and;
- (e) wherein the core is comprised of a substantially greater volume of second material than the volume of first material that comprises the skin; and
- (f) wherein the skin encapsulates an upper surface and sides surface of the core but incompletely encapsulate the core.

2. The synthetic roofing element of claim 1, wherein the skin includes at least one surface having three-dimensional relief therein, simulating a natural material comprising any one of:

- (i) wood shake;
- (ii) tile; and
- (iii) slate.

3. The roofing element of claim 2, wherein the skin of the roofing element encapsulates a surface of the roofing element that is a surface that is weather-exposed in the installed condition of the roofing element on a roof.

4. The roofing element of claim 2, wherein each of the skin and core are constructed of once molten, solidified material.

5. The roofing element of claim 2, wherein the polymer of the first material is selected from the group consisting of:

- (a) polyethylene;
- (b) polypropylene;
- (c) polymethylpentene;
- (d) polybutene;
- (e) polyacrylates; and
- (f) copolymers and/or blends of any of (a) through (e).

6. The roofing element of claim 2, wherein the polymer of the second material is selected from the group consisting of:

- (a) polyvinylchloride;
- (b) polyethylene;
- (c) polypropylene;
- (d) polybutene;
- (e) polymethylpentene;
- (f) polyacrylates;
- (g) polyethyleneterephthalate;
- (h) polybutyleneterephthalate;
- (i) polyethylenenaphthalate;
- (j) ethylene-propylene-diene monomer copolymers; and
- (k) copolymers and/or binary or ternary blends of any of (a) through (j) above.

7. The roofing element of claim 2, wherein the filler of the second material is selected from the group consisting of:

- (a) mineral filler;
- (b) organic filler;
- (c) nanofiller;
- (d) reinforcing filler;
- (e) reinforcing fiber;
- (f) recycled polymer of any of:
  - (i) polyvinylchloride;
  - (ii) polyethylene;
  - (iii) polypropylene;
  - (iv) polybutene;

- (v) polymethylpentene;
- (vi) polyacrylates;
- (vii) polyethyleneterephthalate;
- (viii) polybutyleneterephthalate;
- (ix) polyethylenenaphthalate;
- (x) ethylene-propylene-diene monomer copolymers; and
- (xi) copolymers and/or binary or ternary blends or any combinations of any of (i) through (x) above.

8. The roofing element of claim 2, wherein the first material includes at least one additive therein, with said at least one additive being selected from the group consisting of:

- (a) thermal stabilizers;
- (b) ultraviolet light stabilizers;
- (c) pigments;
- (d) at least one compatibilizer; and
- (e) flame retardants.

9. The roofing element of claim 2, wherein the second material includes at least one additive therein, with said at least one additive being selected from the group consisting of:

- (a) thermal stabilizers;
- (b) ultraviolet light stabilizers;
- (c) pigments;
- (d) at least one compatibilizer; and
- (e) flame retardants.

10. A roof covering comprising a plurality of rigid synthetic roofing elements applied to a roof, side by side, forming a plurality of courses, with roofing elements in given courses comprising underlying courses and having other courses comprising next-overlying courses partially covering the roofing elements in an underlying course, with each roofing element being of the shingle or tile type for exterior application comprising a multi-layer structure having:

- (a) a skin including a first thermoplastic material;
- (b) a core including a second thermoplastic material;
- (c) wherein the first material is a highly weather resistant polymeric material relative to the second material;
- (d) wherein the second material is a polymeric material having filler therein and;
- (e) wherein the core is comprised of a substantially greater volume of second material than the volume of first material that comprises the skin;
- (f) wherein the skin encapsulates an upper surface and sides surface of the core but incompletely encapsulate the core.

11. The roof covering of claim 10, wherein the skins include surfaces having three-dimensional relief therein, simulating natural materials, comprising any one of:

- (i) wood shake;
- (ii) tile; and
- (iii) slate.

12. The roof covering of claim 11, wherein the skins of the roofing elements encapsulate surfaces of the roofing elements that is a surface that is weather-exposed in the installed condition of the roofing elements on a roof.

13. The roof covering of claim 11, wherein each of the skin and core of the roofing elements are constructed of once molten, solidified material.

14. The roof covering of claim 11, wherein the polymer of the first material is selected from the group consisting of:

- (a) polyethylene;
- (b) polypropylene;
- (c) polymethylpentene;
- (d) polybutene;
- (e) polyacrylates; and
- (f) copolymers and/or blends of any of (a) through (e).

**15.** The roof covering of claim **11**, wherein the polymer of the second material is selected from the group consisting of:

- (a) polyvinylchloride;
- (b) polyethylene;
- (c) polypropylene;
- (d) polybutene;
- (e) polymethylpentene;
- (f) polyacrylates;
- (g) polyethyleneterephthalate;
- (h) polybutyleneterephthalate;
- (i) polyethylenenaphthalate;
- (j) ethylene-propylene-diene monomer copolymers; and
- (k) copolymers and/or binary or ternary blends of any of (a) through (j) above.

**16.** The roof covering of claim **11**, wherein the filler of the second material is selected from the group consisting of:

- (a) mineral filler;
- (b) organic filler;
- (c) nanofiller;
- (d) reinforcing filler;
- (e) reinforcing fiber;
- (f) recycled polymer of any of:
  - (i) polyvinylchloride;
  - (ii) polyethylene;
  - (iii) polypropylene;
  - (iv) polybutene;
  - (v) polymethylpentene;
  - (vi) polyacrylates;
  - (vii) polyethyleneterephthalate;
  - (viii) polybutyleneterephthalate;
  - (ix) polyethylenenaphthalate;
  - (x) ethylene-propylene-Diene Monomer Copolymers; and
  - (xi) copolymers and/or binary or ternary blends or any combinations of any of (i) through (x) above.

**17.** The roof covering of claim **11**, wherein the first material includes at least one additive therein, with said at least one additive being selected from the group consisting of:

- (a) thermal stabilizers;
- (b) ultraviolet light stabilizers;
- (c) pigments;
- (d) at least one compatibilizer; and
- (e) flame retardants.

**18.** The roof covering of claim **11**, wherein the second material includes at least one additive therein, with said at least one additive being selected from the group consisting of:

- (a) thermal stabilizers;
- (b) ultraviolet light stabilizers;
- (c) pigments;
- (d) at least one compatibilizer; and
- (e) flame retardants.

**19.** A method of covering a roof comprising providing a plurality of rigid roofing elements and applying said elements to a roof, side by side, in courses, and placing said elements such that the roofing elements in a given course comprise an underlying course, then providing another course that comprises a next-overlying course partially covering the roofing elements in the underlying course, then successively applying additional courses, such that roofing elements in each next-overlying course partially cover roofing elements in a next-underlying course, and wherein the step of providing roofing elements comprises providing synthetic roofing elements of the shingle or tile type for exterior application; and wherein the step of providing roofing elements also includes providing the roofing elements in the form of multi-layer structures, each structure having:

- (a) a skin including a first thermoplastic material;
- (b) a core including a second thermoplastic material;
- (c) wherein the first material is a highly weather resistant polymeric material relative to the second material;
- (d) wherein the second material is a polymeric material having filler therein and;
- (e) wherein the core is comprised of a substantially greater volume of second material than the volume of first material that comprises the skin;
- (f) wherein the skin encapsulates an upper surface and sides surface of the core but incompletely encapsulate the core; and
- (g) wherein the skin includes at least one surface having three-dimensional relief therein, simulating a natural material, comprising any one of:
  - (i) wood shake;
  - (ii) tile; and
  - (iii) slate.

**20.** The method of claim **19**, including the steps of providing each of the skin and core materials in molten form and then solidifying the skin and core materials.

\* \* \* \* \*

UNITED STATES PATENT AND TRADEMARK OFFICE  
**CERTIFICATE OF CORRECTION**

PATENT NO. : 8,206,807 B2  
APPLICATION NO. : 11/742619  
DATED : June 26, 2012  
INVENTOR(S) : Michael L. Friedman et al.

Page 1 of 1

It is certified that error appears in the above-identified patent and that said Letters Patent is hereby corrected as shown below:

Column 3, line 65, reads "as polypropylene tilled with 40-80% by weight of recycled"  
should read -- as polypropylene filled with 40-80% by weight of recycled --

Column 5, line 19, reads "sides surface of the core but incompletely encapsulate"  
should read -- side surfaces of the core but incompletely encapsulates --

Column 6, line 45, reads "sides surface of the core but incompletely encapsulate"  
should read -- side surfaces of the core but incompletely encapsulates --

Column 8, line 33, reads "sides surface of the core but incompletely encapsulate"  
should read -- side surfaces of the core but incompletely encapsulates --

Signed and Sealed this  
Fourteenth Day of August, 2012



David J. Kappos  
Director of the United States Patent and Trademark Office